

# UNITED STATES PATENT OFFICE.

CHARLES H. CAMPBELL, OF CHICAGO, ILLINOIS, ASSIGNOR TO AMERICAN GLUE COMPANY, OF BOSTON, MASSACHUSETTS.

## ADHESIVE AND PROCESS OF MAKING SAME.

1,184,071.

Specification of Letters Patent. Patented May 23, 1916.

No Drawing.

Application filed October 12, 1912. Serial No. 725,432.

*To all whom it may concern:*

Be it known that I, CHARLES H. CAMPBELL, of Chicago, in the county of Cook and State of Illinois, a citizen of the United States, 5 have invented a new and useful Improvement in Adhesives and Processes of Making Same, of which the following is a full, clear, and exact description.

The object of my invention is to provide 10 an animal glue soluble in cold water or water of ordinary temperature.

Various expedients have been resorted to for making a cold-water-soluble animal glue or an animal glue soluble in water of ordinary temperature. Ordinary animal glue 15 possesses a jelly-forming property and also an adhesive strength. For making the glue soluble in water of ordinary temperature the purpose has been to employ an expedient or 20 agent which will destroy the jelly-forming property of the glue. The difficulties with these expedients have been that they have weakened the relative adhesive strength of the glue either by destroying or weakening 25 such strength through chemical reaction upon the glue or by adulterating the glue by reason of the relatively large amount of the agent used. They, also, have the effect of so destroying the jelly-forming property of 30 the glue that when the glue is dissolved it possesses so little body, or in other words, the glue is of such watery consistency, as entirely unsuits it for many purposes.

It is accordingly the further object of my 35 invention to provide a soluble glue possessing a high adhesive strength and in which, also, the jelly-forming property of the glue is not entirely destroyed so that when the glue is dissolved in cold water or water of 40 ordinary temperature it will possess a certain amount of body and will not be of so watery a consistency as will unsuit it for many uses.

The process is as follows: The glue is first 45 treated with a suitable salt of nitric acid and preferably the ordinary chemical commodity potassium nitrate,  $KNO_3$ , although I have found that other salts of nitric acid may be employed with gratifying results. Of the 50 salts of nitric acid suitable for the purpose I find that there need be employed for effecting the desired purpose from three to five

per cent. by weight of the salt of nitric acid used or of the potassium nitrate, to one hundred per cent. by weight of the dry glue. In 55 other words, such amount of the salt is employed as will not injure the adhesive strength of the glue by adulteration or wholly destroy its jelly-forming property. A larger percentage of the agent may be 60 used without chemically injuring the adhesive strength of the glue if by chance a larger amount of the agent be used than is necessary. It will, however, tend to unduly injure the adhesive strength of the glue by 65 adulteration and to destroy its jelly-forming property which I desire to retain in part. The agent is preferably added to the glue liquor (while warm) during the making 70 of the glue and before drying, there being 75 added to the glue liquor three to five per cent. of the agent calculated upon a basis of the dry glue present in the glue liquor. The agent will enter into solution by reason of the water in the glue liquor and will readily 80 act upon the glue, this being preferably facilitated by agitating the liquor. The agent may also be applied to the ordinary dry animal glue. In such case, however, the glue must first be dissolved in the ordinary 85 manner by soaking in water and subsequently heating until the glue has been reduced to a liquid form when the agent is added as before.

According to the process thus far described, the addition of the salt renders the glue soluble in cold water or water of ordinary temperature, but not imparting to it the degree of solubility I desire to obtain if the lesser percentages (three to five per cent. 90 or, thereabout) of the salt are employed and tending to adulterate the glue and to wholly destroy its jelly-forming property if larger percentages are used. These difficulties are overcome, however, by the further continuation 95 of the process. After the lesser percentages of the salt (three to five per cent. or thereabout) have been added to the glue liquor as aforesaid, heat is applied and this preferably during the drying of the glue 100 liquor by the application thereto of artificial heat. I prefer that the degree of heat shall be high and continued for a short period of time, but not so high or continued for so

long a period of time as to injure the adhesive strength of the glue. I find that the best results are obtained by a quick roller drying of the glue liquor in thin films at a 5 temperature of approximately 250° F. for a short period of time, usually in practice about one and one half minutes. The heat may, however, be applied at lower temperatures, for example, 160 to 180° F. preferably 10 for a period of time ranging from ten to fifteen minutes, or even at a lower temperature as from 100 to 120° F. continued for a long period of time, ranging from eighteen to thirty hours, though in neither of these 15 latter cases does one obtain the results obtained from a high degree of heat applied for a short period of time as aforesaid.

The application of the heat to the glue liquor in all cases tends to further but not 20 wholly destroy the jelly-forming property of the glue and to bring out the action of the salt to the best advantage. After the drying of the glue it is ground fine, though this is a preferred step for lessening the time in 25 which the glue will become dissolved in cold water or water of ordinary temperature.

A soluble glue made according to the aforesaid process possesses not only a ready solubility but an adhesive strength greater 30 than its normal strength. It also possesses a body after it has become dissolved which suits it for all purposes of use instead of being of a thin watery consistency as is ordinarily obtained in a soluble glue.

35 What I claim as my invention is:

1. The process of treating animal glue for the purpose of rendering the same soluble at ordinary temperature consisting in treating glue liquor with a suitable salt of nitric 40 acid and subsequently drying the same in the presence of applied heat.

2. A process of making glue soluble at ordinary temperatures which comprises adding a small amount of a substantially neutral, water-soluble nitrate thereto and thereafter applying heat to the dissolved glue in the presence of said nitrate, the amount of heat being substantially equivalent to heating the liquor to a temperature of 250° F., 50 for about one and a half minutes.

3. A process of making glue soluble at ordinary temperature which comprises treating glue liquor with a relatively small amount of a substantially neutral, water- 55 soluble agent, capable in itself of only partially destroying the jelly-forming property of the glue, and subjecting the mixture to heat in amount sufficient to further lessen the jelly-forming property of the glue, and 60 to dry the mass, but insufficient to materially injure the adhesive strength thereof.

4. A process of making glue soluble at ordinary temperature which comprises treating glue liquor with an agent, capable in

itself of only partially destroying the jelly-forming property of the glue, and subjecting the mixture to such high degree of heat for a relatively short period of time as will further lessen the jelly-forming property of the glue, and will dry the glue, but without 70 causing material injury to the adhesive strength thereof.

5. A process of making glue soluble at ordinary temperature which comprises treating glue liquor with an agent, capable in 75 itself of only partially destroying the jelly-forming property of the glue, and afterward drying the mixture by heat applied thereto in amount sufficient to further lessen the jelly-forming property of the glue without 80 materially injuring the adhesive strength thereof.

6. A process of making glue soluble at ordinary temperature which comprises treating glue liquor with an agent, capable in 85 itself of only partially destroying the jelly-forming property of the glue, and afterward drying the mixture by heat applied thereto at such high temperature for a relatively short period of time as will further 90 lessen the jelly-forming property of the glue without materially injuring the adhesive strength thereof.

7. A process of treating glue which comprises adding to glue liquor a substantially 95 neutral, water-soluble nitrate capable of partially destroying the jelly-forming property of the glue, and subsequently drying the same by heat applied thereto.

8. A process of treating glue which comprises heating the glue with not appreciably more than 5% of a soluble nitrate incapable of injuring its adhesive strength, to at least the boiling point of water.

9. A process which comprises treating dissolved glue with a soluble nitrate free from strong acid, and thereafter drying the glue.

10. A process which comprises heating dissolved glue with from 3% to 5% of a soluble nitrate.

11. A process which comprises drying dissolved glue with about 3 to 5% of a soluble nitrate free from strong acid.

12. A process which comprises heating dissolved glue with a relatively small 1 amount of a soluble nitrate free from strong acid sufficiently to dry said mass.

13. A process of treating glue which comprises heating the glue with a nitrate of an alkali, to at least the boiling point of water 1: for a length of time sufficient to substantially dry the mass.

14. A process which comprises treating dissolved glue with a nitrate of an alkali, and thereafter drying the glue.

15. A process which comprises heating dissolved glue with from 3% to 5% of a nitrate of an alkali.

16. A process which comprises drying dissolved glue with about 3 to 5% of a nitrate of an alkali.
17. A dried mixture of glue and a water-soluble nitrate.
18. A dry adhesive comprising glue and a relatively small amount of a nitrate of an alkali.
19. A dry adhesive comprising about 100
- parts of glue and about 3 to 5 parts of an 10 alkali metal nitrate.
20. As an adhesive, a dry, intimate mixture of glue and a soluble nitrate.

CHARLES H. CAMPBELL.

Witnesses:

JOHN E. R. HAYES,  
M. E. FLAHERTY.